

## UNITED STATES PATENT OFFICE

2,494,906

CYAN COMPONENT FOR DIAZOTYPE COLOR  
PROCESS

Sam C. Slifkin and Thaddeus J. Trojnar, Bing-  
hamton, N. Y., assignors to General Aniline &  
Film Corporation, New York, N. Y., a corpora-  
tion of Delaware

No Drawing. Application June 6, 1947,  
Serial No. 753,036

4 Claims. (Cl. 95--6)

1

The present invention relates to sensitized diazotype materials for the diazotype color process which when exposed through a cyan separation positive and developed yield greenish blue images of high intensity.

It has been suggested that the diazotype process be utilized for the purpose of manufacturing natural color prints. The method suggested involved printing separation positives in the primary colors on separate transparent plastic film layers, dry-developing the layers and transposing the layers in register to produce a color print.

This process, however, was found to be unsatisfactory primarily because the sensitized compositions used for producing the cyan records yielded images too blue in color. Inasmuch as the cyan record is the key image record just as in color photography the decided blue nature of this record led to color distortion. This phenomenon which also manifests itself in three-color photography as may be seen from Frohlich et al. U. S. Patent No. 2,357,394 militated against the adoption of the aforementioned process despite the simplicity inherent therein.

We have now discovered that the objections referred to above can be completely avoided and cyan records blue-green in color and of high intensity can be obtained if there can be used as the coupling component for the layer in which the cyan separation is to be recorded a 1-hydroxy-naphthalene sulfonic acid containing in the 8-position a hydroxyl group or an amino or substituted amino group. The employment of such coupling components in the sensitizing compositions used to produce the cyan records in the diazotype color process and the processing of carriers bearing such compositions constitute the purposes and objects of the present invention.

The coupling components contemplated herein are typified by the following structural formula:



in which R is hydroxyl, amino, acylamino, such as, acetylamino, propionylamino, butyrylamino, benzoylamino, and the like, alkylamino, such as,

2

methylamino, dimethylamino, ethylamino, diethylamino, and the like, or arylamino, such as, phenylamino, di-phenylamino, and the like.

Examples of compounds embraced by this formula and which we have found to be satisfactory for our purposes are:

- 1. 8-dihydroxy-naphthalene-3-sulfonic acid
- 1. 8-dihydroxy-naphthalene-4-sulfonic acid
- 10 1-hydroxy-8-amino-naphthalene-2-sulfonic acid
- 1-hydroxy-8-amino-naphthalene-4-sulfonic acid
- 1-hydroxy-8-amino-naphthalene-6-sulfonic acid
- 1-hydroxy-8-amino-naphthalene-3-sulfonic acid
- 1-hydroxy-8-amino-naphthalene-5-sulfonic acid
- 15 1 - hydroxy - 8 - acetylamino - naphthalene - 3- sulfonic acid
- 1 - hydroxy - 8 - propionylamino - naphthalene - 4-sulfonic acid
- 20 1 - hydroxy - 8 - benzoylamino - naphthalene - 7- sulfonic acid
- 1 - hydroxy - 8 - methylamino - naphthalene - 5- sulfonic acid
- 1 - hydroxy - 8 - dimethylethylamino - naphthalene-6-sulfonic acid
- 25 1 - hydroxy - 8 - butyrylamino - naphthalene - 5- sulfonic acid
- 1 - hydroxy - 8 - phenylamino - naphthalene - 4- sulfonic acid

The 1.8-dihydroxy-naphthalene sulfonic acids and the 1-hydroxy-8-amino-naphthalene sulfonic acids are well known compounds. The acyl derivatives mentioned above may be prepared by treatment of the 1-hydroxy-8-amino-naphthalene sulfonic acids with the anhydrides of the acids involved just as in the preparation of, for instance, acetyl J acid. Generally, the 1-hydroxy-8-amino-naphthalene sulfonic acids in which the amino group is substituted by alkyl or aryl may be prepared by alkylation and arylation, just as in the preparation of, for instance, dimethyl-2-amino-8-naphthol-6-sulfonic acid or of phenyl J acid.

The diazo component which is utilized in the sensitizing composition may be any of those generally employed in the diazo-type art although we prefer the N-substituted p-phenylenediamines. While the diazos are preferably employed in the form of the zinc chloride double salts they may likewise be utilized as such or in the form of their double salts with cadmium

chloride, tin chloride or the like, or in the form of the fluoro-borates or the alkyl or aryl sulfonates, such as, the methyl, ethyl, propyl, phenyl and the like sulfonates.

Examples of diazos which we have found to yield excellent results are those derived from the following compounds:

p-amino-N-diethyl-o-toluidine  
4-diethylamino-o-phenetidine  
p-(N-ethyl-N-hydroxyethylamino)-o-toluidine

The sensitizing compositions in addition to the diazo compound and the azo coupling component also contain the usual adjuncts designed to effect stabilization, such as, thiourea, thiosinamine, and the like, and to retard precoupling, such as, citric acid, tartaric acid, boric acid, and the like.

The components prior to application to the base are dissolved in suitable solvents, such as, water or mixtures of water and a low molecular weight alcohol, i. e., methyl alcohol, ethyl alcohol, and the like.

The base to which the sensitizing compositions are applied may be a sheet, film, or the like, of any transparent film-forming material preferably a cellulose ester, such as, cellulose acetate, cellulose propionate, cellulose acetate propionate, and the like.

The sensitized base is utilized in the manner outlined above, that is, by exposure under a desired cyan separation positive by U. V. light and development by ammonia fumes.

The following examples serve to illustrate the invention but it is to be understood that the invention is not restricted thereto:

#### Example I

A cellulose acetate film is coated with a solution of the following components:

|                                           |       |    |
|-------------------------------------------|-------|----|
| Water                                     | cc    | 50 |
| Alcohol                                   | cc    | 50 |
| Citric acid                               | grams | 5  |
| Thiourea                                  | do    | 2  |
| 1.8-dihydroxy-naphthalene-4-sulfonic acid | grams | 2  |

The zinc chloride double salt of the diazo from 4-diethylamino-o-phenetidine grams 4

When dried and exposed to U. V. light under a selected cyan separation positive and developed in the usual way with ammonia vapor, a greenish-blue positive reproduction of high density is obtained.

#### Example II

The procedure is the same as in Example I excepting that 1-hydroxy-8-amino-naphthalene-4-sulfonic acid is substituted for the dihydroxy-naphthalene sulfonic acid. By working up the film as in Example I, a greenish-blue record of high density and contrast is obtained.

#### Example III

The procedure is the same as in Example I excepting that 1-hydroxy-8-acetylamino-naph-

thalene-4-sulfonic acid is substituted for the dihydroxy-naphthalene sulfonic acid. Here again, the processing of the resulting film leads to greenish-blue positives of high density.

5 We claim:

1. Light sensitive diazotype material for use in producing a cyan record in the diazotype color process comprising a transparent base carrying as a light sensitive diazo compound a diazotized 10 p-phenylene-diamine in which one of the amino groups is di-substituted by members selected from the class consisting of alkyl and hydroxyalkyl and as the azo component a compound of the following formula:

15



20

wherein R is a member selected from the class consisting of hydroxyl, amino, acylamino, alkylamino, and arylamino.

25 2. The article as defined in claim 1 in which the azo coupling component is 1.8-dihydroxy-naphthalene-4-sulfonic acid.

30 3. The article as defined in claim 1 wherein the light sensitive diazo compound is the zinc chloride double salt of the diazo from 4-diethylamino-o-phenetidine and the azo coupling component is 1.8-dihydroxy-naphthalene-4-sulfonic acid.

35 4. The process of producing cyan diazotype prints capable of transmitting both green and blue light which comprises sensitizing a transparent base with a composition containing as a light sensitive diazo compound a diazotized p-phenylene-diamine in which one of the amino groups is di-substituted by members selected from the class consisting of alkyl and hydroxyalkyl and 40 as a coupling component a compound of the following formula:

45



wherein R is a member selected from the class consisting of hydroxyl, amino, acylamino, alkylamino, and arylamino, exposing the sensitized base through a cyan separation positive by U. V. light and developing the exposed material with ammonia vapor.

55

SAM C. SLIFKIN.  
THADDEUS J. TROJNAR.

#### REFERENCES CITED

The following references are of record in the file of this patent:

#### UNITED STATES PATENTS

| Number    | Name            | Date          |
|-----------|-----------------|---------------|
| 1,710,455 | Langguth et al. | Apr. 23, 1929 |
| 2,375,366 | Jacobus         | May 8, 1945   |

60  
65